# EUROPEAN PATENT SPECIFICATION

(11) **EP 0 370 441 B1**
(45) Date of publication and mention of the grant of the patent: **09.02.1994**
(21) Application number: 89121466.0
(22) Date of filing: 20.11.1989
(51) Int. Cl.: B41M 5/26

(54) **Image-receiving sheet for thermal transfer printing with an intermediate layer containing fine particles of thermosetting resin and fine particles of polyolefin resin**
Bildempfangsschicht für thermischen Übertragungsdruck mit einer Zwischenschicht, die feinkörnige Teilchen von hitzehärtbarem Harz und feinkörnige Teilchen von Polyolefinharz enthält
Feuille réceptif pour l'impression thermique par transfert avec une couche intermédiaire contenant de fines particules d'une résine thermoplastique et d'une résine polyoléfine

(30) Priority: 21.11.1988 JP 294377/88
(43) Date of publication of application: 30.05.1990
(73) Proprietor: KANZAKI PAPER MANUFACTURING CO., LTD., Chiyoda-ku, Tokyo-to (JP); DAI NIPPON INSATSU KABUSHIKI KAISHA, Tokyo 162 (JP)
(72) Inventor: Okumura, Yoshitaka, Kyoto-shi Kyoto (JP); Watanabe, Kazuo, Itami-shi Hyogo-ken (JP); Kondo, Hiromasa, Ikoma-shi Nara-ken (JP); Egashira, Noritaka, Ichikawa-shi Chiba-ken (JP); Satake, Naoto, Shinjuku-ku Tokyo (JP)
(74) Representative: Kraus, Walter, Dr.

(56) References cited:
- PATENT ABSTRACTS OF JAPAN vol. 11, no. 16 (M-554)(2463) 16 January 1987; JP-A-61 192595 (RICOH CO LTD) 27 August 1986.
- PATENT ABSTRACTS OF JAPAN vol. 10, no. 342 (M-536)(2398) 19 November 1986; JP-A-61 144394 (DAINIPPON PRINTING CO LTD) 02 July 1986.
- PATENT ABSTRACTS OF JAPAN vol. 5, no. 10 (M-51)(682) 22 January 1981; JP-A-55 140590 (RICOH K.K.) 04 November 1980.
- PATENT ABSTRACTS OF JAPAN vol. 11, no. 166 (M-593)(2613) 28 May 1987; JP-A-61 295085 (DAINIPPON PRINTING CO LTD) 25 December 1986.
- PATENT ABSTRACTS OF JAPAN vol. 10, no. 100 (M-470)(2157) 16 April 1986; JP-A-60 236794 (MATSUSHITA DENKI SANGYO K.K.) 25 November 1985.

## Description

The present invention relates to an improved image-receiving sheet for thermal transfer printing in which a thermally sublimable dye is used. More particularly, the present invention relates to an improved image-receiving sheet for thermal transfer printing which has an improved intermediate layer containing fine particles of thermosetting resin and fine particles of polyolefin resin and which exhibits an improved recording sensitivity and provides excellent printed images with no missing dot.

Thermal printing systems in which printed images are obtained upon reception of input signals are made up of a relatively simple apparatus and are inexpensive and low in noises. In view of this, they have increasing utility in various fields such as facsimiles, terminal printers for electronic computers, printers for measuring instruments, video printers, and the like.

As the recording medium to be used in these thermal printing systems, there has been generally used a so-called spontaneous developing heat sensitive paper having a recording layer capable of causing a physical or chemical change upon application of heat to provide color development. However, the spontaneous developing heat sensitive paper of the color developing type has disadvantages that it is liable to undesirably cause color development during the fabrication process or during storage; and the images printed on the paper are poor in storage stability and they are apt to fade on contact with organic solvents or chemicals.

In order to improve the above situation, there has been proposed a printing system wherein a recording medium in which a coloring material such as a dye or colorant is utilized is used in stead of the foregoing spontaneous developing heat sensitive paper, for example, as disclosed in JP-A-51(1976)-15446. In the printing system disclosed in this publication, a sheet comprising a substrate such as a paper or polymer film and a colorant layer containing the coloring material (which is in the solid or semi-solid state at ordinally temperature) being formed on the substrate is firstly provided, and this sheet and a recording sheet are superposed so as to make the colorant layer contacted with the recording sheet and heated from the non-faced side of the former sheet by a heating means such as a thermal head to transfer the coloring material in the colorant layer on the recording sheet upon the electric signals provided by the heating means, whereby images corresponding to image information are recorded on the recording sheet.

In the above printing system, the coloring material in the colorant layer is caused to melt, evaporate or sublimate by application of heat and transferred on the recording sheet, thereby forming a record image by adhesion, adsorption or reception of the coloring material on the recording sheet. In view of this, this printing system has been evaluated as being advantageous with a view point that there can be used an ordinary paper (wood free paper) as the recording sheet. Further, as for this printing system, when a sublimable dye is used as the coloring material, there can be obtained a printed image excelling in tone reproduction. In order to develop this advantage in the full-color printing, various studies have been made.

However, there are disadvantages for the foregoing printing system wherein an ordinary paper (wood free paper) is used as the recording sheet that sufficient dye-reception hardly occur to cause such printed images which are poor in color density (optical density) and those image will be markedly discolored as time lapses.

To avoid this, there has been proposed the use of an image-receiving sheet having an image-receiving layer containing a thermosetting resin as the main constituent which is formed on a substrate as disclosed in JP-A-57(1982)-107885 or US-A-3,601,484.

The use of this image-receiving sheet is effective in somewhat improving the recording sensitivity and storage-ability. However, there still remains a problem that when an ordinary paper (wood free paper) is used as the substrate, it is difficult to provide a desirable image-receiving layer containing a thermosetting resin as the main constituent of uniform thickness with the paper and thus, the resulting image-receiving sheet unavoidably becomes such that is poor in the recording sensitivity and provides undesirable images inferior in the quality.

In order to eliminate the above problem, there has been proposed another image-receiving sheet having an intermediate layer comprising a thermosetting resin which is disposed between a substrate and an image-receiving layer as disclosed in JP-A-60(1985)-236794 or JP-A-61(1986)-144394.

This image-receiving sheet is so designed that its image-receiving layer can be effectively contacted with the dye layer of the dye transfer sheet to prevent occurrence of negative phenomena such as air-gap upon printing, and it exhibits an improved recording sensitivity and provides improved record images.

In addition, there has been proposed a further image-receiving sheet having an intermediate layer containing fine particles of a specific polyolefin resin which is disposed between a substrate and an image-receiving layer by, among others, four of the coinventors of the present invention as disclosed in US-A-4,837,200. The use of this image-receiving sheet is effective especially in obtaining desirable recorded images free of missing transfer portion.

The present inventors have made various studies on the foregoing image-receiving sheets having an intermediate layer in order to make further improvements therefor.

As a result, it has been found that any of said image-receiving sheets is still accompanied with a disadvantageous point that it is necessary to use a sufficiently white sheet as the substrate and otherwise, it is extremely difficult to obtain a sufficiently white image-receiving sheet which is practically acceptable as a recording sheet, since the intermediate layer is insufficient in the covering power particularly when it is formed by the use of fine particles of a single resin, and because of this, there is a limit for the kind of the substrate to be used in any of the foregoing cases.

The present inventors have tried to incorporate into the intermediate layer an inorganic pigment such as calcium carbonate, talc, kaolin, titanium oxide, aluminum hydroxide, zinc oxide, etc., or an organic pigment, wherein an ordinary paper was used as the substrate, in order to eliminate the foregoing disadvantageous point. As a result, it has been found that the resulting image-receiving sheet rather becomes accompanied with a further disadvantage of causing reduction in the optical density and also in the quality of images as printed and this situation becomes significant as the amount of such pigment to be incorporated in the intermediate layer increases.

Standing on the above findings, the present inventors have made further studies in order to provide a desirably improved image-receiving sheet comprising a substrate, an intermediate layer and an image-receiving layer for thermal transfer printing for use in the printing system wherein a coloring material, particularly a sublimable dye is thermally transferred.

As a result, it has been found that when the intermediate layer is formed by using fine particles of a specific thermosetting resin and fine particles of a polyolefinic resin in combination, there can be obtained a desirable image-receiving sheet having an improved opacity for the intermediate layer. And as a result of evaluating the image-receiving sheet thus obtained with various items required for an image-receiving sheet to be practically applicable, it has been found that it is extremely high in the recording sensitivity and provides high quality record images excelling in resolution, clearness and optical density and which are not accompanied with any missing dots. It has been also found that the foregoing image-receiving sheet is satisfactory in whiteness and opacity even in the case where an ordinary paper (wood free paper) is used as the substrate and it can be mass-produced with a reduced cost.

The present invention has been accomplished based on the above findings.

An object of the present invention is to provide an improved image-receiving sheet for thermal transfer printing which is free of the foregoing problems which are found on the known image-receiving sheet and which enables one to form beautiful record images of high optical density.

Another object of the present invention is to provide an improved image receiving sheet which is satisfactory in whiteness and opacity even upon using an ordinary paper (wood free paper) as the substrate.

A further object of the present invention is to provide an improved image-receiving sheet which exhibits an excellent recording sensitivity and provides high quality record images excelling in resolution and clearness which are not accompanied with any missing dots.

The present invention attains the above objects and it contemplates to provide an improved image-receiving sheet for thermal transfer printing for use in the printing system wherein a sublimable dye is thermally transferred.

Accordingly the present invention provides an image-receiving sheet for thermal transfer printing comprising a substrate, an intermediate layer and an image-receiving layer, said intermediate layer and said image-receiving layer being disposed in this order on said substrate, which is characterized in that said intermediate layer comprises a layer containing (a) fine particles of one or more kinds of thermosetting resins and/or (b) fine particles of one or more kinds of other resins than said thermosetting resins, having a softening point of higher than 150°C and (c) fine particles of a polyolefin resin as the main constituents.

The image-receiving sheet of the present invention comprises a substrate, an intermediate layer and an image-receiving layer, said intermediate layer and said image-receiving layer being disposed in this order on said substrate, and said intermediate layer containing fine particles of a thermosetting resin and/or fine particles of a resin having a softening point of more than 150°C and fine particles of a polyolefin resin.

The image-receiving sheet of the present invention is characterized by having a specific intermediate layer containing (a) fine particles of a thermosetting resin and/or (b) fine particles of a resin having a softening point of higher than 150°C and (c) fine particles of a polyolefin resin.

The fine particles of a thermosetting resin (a), the fine particles of a resin having a softening point of higher than 150°C (b) and the fine particles of a polyolefin resin (c) will be hereinafter abbreviated simply as "thermosetting resin fine particle", "high softening point resin fine particle" and "polyolefin resin fine particle", respectively.

As for the polyolefin resin which is of a low softening point and flexible and which is capable of contributing to improving the recording sensitivity and the quality of an image printed when used in the image-receiving sheet, there can be mentioned, for example, polyethylene, polypropylene, polybutene-1, polyisobutylene, polypentene-1, polyhexene-1, poly-3-methylbutene-1, poly-4-methylpentene-1, poly 5-methylhexene-1, etc., and copolymers of two or more of these polymers.

These polyolefin resins are commercially available in the form of fine particles.

These polyolefin resin fine particles are not soluble in organic solvents and because of this, they can be desirably used in the formation of an intermediate layer not only in the case where an image-receiving layer is formed in the organic solvent system or in the aqueous system.

However, the softening point of any of the foregoing polyolefin resin fine particles is in the range of 40 to 150°C. Therefore, they are problematic upon forming the intermediate layer with the use of any of them since they are softened and finally melted with the heat applied in the process of preparing an image-receiving sheet. Thus, the resulting intermediate layer unavoidably becomes such that is inferior in the coverage.

In view of the above, in the present invention, at least a member selected from the group consisting of thermosetting resins and high softening point resins respectively in the form of fine particles (these resins will be collectively called "high softening point resins" hereinafter) is used together with the polyolefin resin fine particle.

The high softening point resin fine particles and the thermosetting resin fine particles are hardly softened or melted by the action of heat applied in the process of preparing an image-receiving sheet. In addition to this, when it is used together with the polyolefin resin fine particle for the formation of the intermediate layer, the resulting intermediate layer becomes provided with a desirable whiteness and a desirable opacity. Further in addition, the resulting intermediate layer becomes to have a such a layer structure that contains a plurality of minute cavities. For these reasons, the resulting image-receiving sheet such that have a intermediate layer becomes to have a desirable heat-resistance and provide a significant effect of enhancing the printing density, whereby obtaining extremely high quality printed images since it is free of such a disadvantage that loss of energy occurs due to endothermal phenomenon caused by the melting of the constituent fine particles upon printing, which is often found on the known image-receiving sheet.

As high softening point resin fine particles and thermosetting resin fine particles which can be used in the present invention fine particles of various cross linked resins and fine particles of various thermosetting resins can be mentioned. Specific examples of the cross linked resin fine particles are, for example, fine particles of cross linked styrenic resins, fine particles of cross linked styrene-acrylic resins, etc. Specific examples of the thermosetting resin fine particle are phenol resin fine particle, urea resin fine particle, melamine resin fine particle, aryl resin fine particle, polyimide resin fine particle, benzoguanamine resin particle, etc.

The term "softening point" in the present invention denotes the temperature when a high molecular material converts from the original solid state into a state of low elastic modules i.e. a so-called gum state as the temperature heightens and then it is softened and melted as the temperature further heightens.

In the present invention, the polyolefin resin fine particle and the high softening point resin fine particle are mixed at an appropriate mixing ratio in the range where the characteristics of the intermediate layer are not hindered.

However, in general, the amount of the high softening point resin fine particle to be mixed with the polyolefin resin fine particle is desired to be preferably in the range of from 5 to 90% by weight, more preferably in the range of from 10 to 60% by weight, respectively versus the total of the high softening point resin fine particle and the polyolefin resin fine particle. When it is less than 5% by weight, the resulting intermediate layer becomes to have insufficient whiteness and opacity. On the other hand, when it exceeds 90% by weight, negative reduction will be caused for the optical density and the quality of an image as printed.

The intermediate layer according to the present invention may be formed as follows. That is, firstly, an aqueous emulsion containing the foregoing high softening point resin fine particle and the foregoing polyolefin resin fine particle is prepared. Then, a synthetic polymer adhesive such as polyacrylic acid ester, styrene-butadiene copolymer or polyvinyl acetate and/or a natural adhesive such as starch or casein are dispersed into the foregoing aqueous emulsion to obtain a coating composition. The coating composition thus obtained is applied onto the surface of a substrate in a predetermined amount by known coating means such as wire-bar coater, air-knife coater, blade coater, gravure-roll coater, curtain coater, etc., to thereby form a liquid coat to be the intermediate layer, followed by air-drying.

Thus, there can be formed the intermediate layer as desired.

As for the amount of the foregoing coating composition to be applied onto the surface of a substrate for forming the intermediate layer, it is desired to be preferably 1 g/m² or more, more preferably in the range of from 3 to 30 g/m² on a dry basis.

In a preferred embodiment, the intermediate layer thus formed is graduated with heat or pressure using a proper graduation means such as super calender after or prior to forming the image-receiving layer thereon. In this case, the recording sensitivity of the resulting image-receiving sheet is markedly improved to provide a significantly high quality printed image.

For the image-receiving layer to be formed on the intermediate layer in the present invention, there is not any particular restriction. However, it is desired to be comprised of a thermosetting resin layer capable of exhibiting an effective dye-receptivity for a sublimable dye.

As the thermosetting resin to constitute the image-receiving layer, there can be mentioned, for example, polymers of vinyl monomer such as styrene, vinyltoluene, acrylic ester, methacrylic ester, acrylonitrile, vinyl chloride, vinyl acetate, etc.; copolymers of these monomers; condensed polymers such as polyester, polyamide, polycarbonate, polysulfone, epoxy resin, polyurethane, etc.; and cellose resins.

These thermosetting resins may be used alone or in combination of two or more of them.

In case where necessary, the image-receiving layer in the present invention may contain one or more of other resins selected from the group consisting of methyl cellulose, ethyl cellulose, hydroxypropyl cellulose, starch, polyvinyl alcohol, polyamide resin, phenol resin, melamine resin, urea resin, urethane resin, epoxy resin, silicone resin, etc. in an amount in the range where the effects of the present invention are not hindered.

Further, the image-receiving layer in the present invention may contain a reactive compound such as polyvalent isocyanate compound, epoxy compound or organometallic compound. In this case, the quality of the image-receiving layer is improved.

Further in addition, it is possible to incorporate a proper auxiliary into the image-receiving layer aiming at providing it with an improved writeability. As such auxiliary, there can be mentioned, for example, inorganic or organic pigments such as ground calcium carbonate, precipitated calcium carbonate, talc, clay, natural or synthetic silicate, titanium oxide, aluminum hydroxide, zinc oxide, urea-formaldehyde resin, etc.; ultraviolet ray absorbing agents; antioxidants; antistatic additives; releasing agents; lubricants, etc. These auxiliaries may be used alone or in combination of two or more kinds of them.

The image-receiving layer in the present invention may be properly formed in the manner similar to the foregoing manner of forming the intermediate layer. For instance, the image-receiving layer is formed on the previously formed intermediate layer by using a coating composition containing the foregoing thermosetting resin or a coating composition containing, in addition to the foregoing thermosetting resin, the foregoing pigment or/and the foregoing auxiliary, applying said coating composition onto the surface of the previously formed intermediate layer in a predetermined amount by the foregoing coating means to therby form a liquid coat and air-drying said liquid coat.

The amount of the foregoing coating composition to be applied to form the image-receiving layer is properly determined depending upon the use purpose of the resulting image-receiving sheet. However, in general, it is desired to be in the range of 2 to 15 g/m² on a dry basis.

As the substrate of the image-receiving sheet according to the present invention, a wood free paper, a synthetic paper or a polymer film can be selectively used. Among these, the wood free paper is most preferred since it excels not only in heat resisting property but also other thermal properties. The wood free paper used in the present invention includes papers manufactured under acidic conditions, neutral conditions or alkaline conditions which are comprised chiefly of cellulose pulp and added with a wet strength agent, sizing agent, filler such as inorganic or organic pigment, etc.

The wood free paper also includes those papers manufactured by size-pressing the above papers with oxidized starch or the like and other papers having an improved surface physical property manufactured by providing the above papers with a precoat layer containing a pigment such as clay as the main constituent.

Other than those above mentioned, a No. 1 grade coated paper, a coated paper or a cast coated paper can be more suitably used as the substrate in the present invention.

In the present invention, such a thin heat-resistant protective layer containing a silicone resin as the main constituent, capable of permeating a sublimable dye as disclosed in Japanese Unexamined Patent Publication Sho. 59(1984)-165686 or Sho. 61(1986)-27290 may be disposed on the surface of the image-receiving layer. In this case, the dye or the dye layer can be prevented from directly transferring to the image-receiving layer.

As above described, the image-receiving sheet for thermal transfer printing to be provided according to the present invention exhibits marked performances when used in the thermal transfer printing system wherein a dye transfer sheet containing a thermally sublimable dye is used.

The thermally sublimable dye in the present invention includes such dyes that do not cause transfer even on contact with the image-receiving sheet under ordinary handling conditions but cause transfer, for the first time, with application of heat of 60°C or more by way of melting, vaporization, sublimation and the like.

As such dye, there can be mentioned, for example, disperse system dyes such as azo series dyes, nitro series dyes, anthraquinone series dyes, quinoline series dyes, etc.; basic dyes such as triphenylmethane series dyes, fluoran series dyes, etc.; and oil soluble dyes.

The image-receiving sheet for thermal transfer printing to be provided according to the present invention is usable not only in the thermal transfer printing system wherein contact heat caused, for example, by a heating plate or thermal head of thermal printing unit is utilized but also in other thermal printing system wherein indirect contact heat with the use of infrared lamp, YAG laser or carbon dioxide gas laser is utilized.

### PREFERRED EMBODIMENTS OF THE INVENTION

The advantages of the present invention are now described in more detail by reference to the following Examples and Comparative Examples, which are provided here for illustrative purposes only, and are not intended to limit the scope of the present invention.

Unless otherwise indicated, parts and % signify parts by weight and % by weight respectively.

### EXAMPLE 1

A coating composition having a solid content of 40% for the intermediate layer was firstly prepared by mixing 250 parts of thermosetting benzoguanamine resin fine particles of 2 µm in particle size (trade name: EPOSTAR-EPS-MS, produced by Nippon Syokubai Kagaku Kogyo Co., Ltd.), 600 parts of polyolefin resin fine particles of 5 µm in particle size (softening point: 54°C, solid content: 40%)(trade name: CHEMIPEARL A-100, produced by Mitsui Petrochemical Industries Co., Ltd.) and 150 parts of styrene-butadiene copolymer emulsion (solid content: 48%)(trade name: L-1690, produced by Asahi Chemical Industry Co., Ltd.) as a binder to obtain a mixture and adding water to the mixture.

The coating composition thus obtained was applied onto a No. 1 grade coated paper of 128 g/m² (trade name: SA-KINFUJI, produced by Kanzaki Paper Manufacturing Co., Ltd.) in an amount to be 15 g/m² when dried to form a liquid coat comprising said coating composition on said paper by the use of a wire-bar coater, followed by air-drying, to thereby form an intermediate layer.

Then, a coating composition for the image-receiving layer which was prepared by dissolving 20 parts of polyester resin (trade name: VYLON-200, produced by Toyobo Co., Ltd.) in an solvent composed of 40 parts of methyl ethyl ketone, 40 parts of toluene and 20 parts of cyclohexanone to obtain a solution and adding to the solution 0.3 parts of amino denatured silicone oil (trade name: KF-393, produced by Shinetsu Chemical Co., Ltd.) and 0.3 parts of epoxy denatured silicone oil (trade name: X-33-343, produced by Shinetsu Chemical Co., Ltd.) was applied onto the surface of the previously formed intermediate layer in an amount to be 4 g/m² when dried in the same manner as in the case of forming the intermediate layer to form a liquid coat. The liquid coat thus formed was then subjected to air-drying and curing at 120°C for 5 minutes.

The resultant was graduated at a linear pressure of 200 kg/cm by means of a super calender comprising a metal roll having a mirror ground surface and a elastic roll. Thus, there was obtained an image-receiving sheet for thermal transfer printing of the present invention.

### EXAMPLE 2

The procedures of Example 1 were repeated, except that as the coating composition for the intermediate layer, a coating composition having a solid content of 30% prepared by mixing 35 parts of thermosetting urea formaldehyde resin fine particles of 5 to 6 µm in secondary particle size (trade name: PERGOPAK M2, produced by Ciba Geigy Co., Ltd.), 850 parts of polyolefin resin fine particles (trade name: CHEMIPEARL A-100) and 115 parts of styrene-butadiene copolymer emulsion of 50% in a solid content (trade name: JSR-0530, produced by Japan Synthetic Rubber Co., Ltd.) as a binder to obtain a mixture and adding water to the mixture was used, to thereby an image-receiving sheet for thermal transfer printing of the present invention.

### EXAMPLE 3

The procedures of Example 1 were repeated, except that as the coating composition for the intermediate layer, a coating composition having a solid content of 40% prepared by mixing 570 parts of cross linked styrenic resin fine particles of 0.3 to 0.4 µm in particle size and having a softening point of 156°C (solid content: 20%)(trade name: GRANDOLL PP-5491, produced by Dainippon Ink & Chemicals Inc.), 285 parts of polyolefin resin fine particles (trade name: CHEMIPEARL A-100) and as a binder, 145 parts of styrene-butadiene copolymer emulsion having a solid content of 48% (trade name: L-1690) to obtain a mixture and adding water to the mixture, to thereby obtain an image-receiving sheet for thermal transfer printing of the present invention.

### Comparative Example 1

A comparative image-receiving sheet for thermal transfer printing was prepared by repeating the procedures of Example 1, except that as the coating composition for the intermediate layer, a coating composition composed of 890 parts of polyolefin resin fine particles (trade name: CHEMIPEARL A-100) and 110 parts of styrene-butadiene copolymer emulsion (trade name: JSR-0530) was used.

### Comparative Example 2

A comparative image-receiving sheet for thermal transfer printing was prepared by repeating the procedures of Example 1, except that as the coating composition for the intermediate layer, a coating composition having a solid content of 40% prepared by mixing 865 parts of thermosetting benzoguanamine resin fine particles (trade name: EPOSTAR EPS-MS) and 135 parts of styrene-butadiene copolymer emulsion (trade name: L-1690) to obtain a mixture and adding water to the mixture was used.

### Comparative Example 3

A comparative image-receiving sheet for thermal transfer printing was prepared by repeating the procedures of Example 1, except that as the coating composition for the intermediate layer, a coating composition having a solid content of 40% prepared by mixing 250 parts of anatase type titaium oxide fine particles (trade naem: FA-55W, produced by Furukawa Mining Co., Ltd.), 600 parts of polyolefin resin fine particles (trade name: CHEMIPEARL A-100) and 150 parts of styrene-butadiene copolymer emulsion (trade name: L-1690) to obtain a mixture and adding water to the mixture was used.

### Comparative Example 4

A comparative image-receiving sheet for thermal transfer printing was prepared by repeating the procedures of Example 1, except that as the coating composition for the intermediate layer, a coating composition having a solid content of 40% prepared by mixing 445 parts of polyethylene resin fine particles of 3 µm in particle size and having a softening point of 132°C (solid content: 40%) (trade name: CHEMIPEARL W-300, produced by Mitsui Petrochemical Industries Co., Ltd.), 445 parts of polyolefin resin fine particles (trade name: CHEMIPEARL A-100) and 110 parts of styrene-butadiene copolymer emulsion (trade name: JSR-0530) to obtain a mixture and adding water to the mixture was used.

### EVALUATION

The seven image-receiving sheets obtained in Examples 1 to 3 and Comparative Examples 1 to 4 were evaluated.

In the evaluation of each of the image-receiving sheets, there was used a thermal dye-transfer sheet which was prepared in the way as below described.

That is, 0.45 parts of a blue thermally sublimable disperse dye (trade name: KST-B-714, produced by Nippon Kayaku Co., Ltd.) and 0.4 parts of polyvinyl butyral resin (trade name: Eslec BX-1, produced by Sekisui Chemical Co., Ltd.) were dissolved in a solvent composed of 4.6 parts of methyl ethyl ketone and 4.6 parts of toluene to obtain an ink composition for the formation of a thermal dye-transfer layer. The composition thus obtained was applied onto a 6 µm thick polyethylene terephthalate film whose reverse side has been subjected to heat-resisting treatment, in an amount to be 1.0 g/m² when dried by means of a wire bar coater and dried to obtain a thermal dye-transfer sheet.

The thermal dye-transfer sheet thus obtained was superposed on the image-receiving sheet sample to be evaluated, followed by printing with application of heat through a thermal head, where a voltage was impressed under conditions of 12 V and 2 to 8 m sec for evaluating the recording sensitivity of the image-receiving sheet sample and the quality of an image as printed.

In addition, the opacity and whiteness were evaluated for each of the image-receiving sheet samples.

The above evaluations were made in the following manners.

### Evaluation of the recording sensitivity:

The image obtained was measured by Macbeth Reflection Densitometer (product of Macbeth Corp., U.S.A.) with its optical density. The results obtained were evaluated with reference to the previously provided standard curve of the recording sensitivity.

### Evaluation of the quality of an image obtained:

This evaluation was conducted by observing the image obtained by eyes with the use of a magnifier with a 25 times magnification.

### Evaluation of the opacity:

The image-receiving sheet sample was measured in accordance with the manner of JIS-P-8138 to obtain a value. And its opacity was evaluated based on the resultant value.

### Evaluation of the whiteness:

The image-receiving sheet sample was set to Elrepho Whiteness Measuring Device (product of Karl Zweis Co., Ltd.) to thereby evaluate its whiteness.

The evaluated results were collectively shown in Table 1.

From the results shown in Table 1, it has been recognized that any of the image-receiving sheets obtained in Examples 1 to 3 is good or excellent with respect to any of the evaluation items and provides satisfactory results in practical use.

## Claims

1. An image-receiving sheet for thermal transfer printing comprising a substrate, an intermediate layer and an image-receiving layer, said intermediate layer and said image-receiving layer being disposed in this order on said substrate, characterized in that said intermediate layer comprises a layer containing
(a) fine particles of one or more kinds of thermosetting resins and/or
(b) fine particles of one or more kinds of other resins than said thermosetting resins, having a softening point of higher than 150°C and
(c) fine particles of a polyolefin resin as the main constituents.

2. An image-receiving sheet for thermal transfer printing according to claim 1, wherein the amount of the fine particles (a) contained in the intermediate layer is in the range of from 5 to 90% by weight versus the total amount of the fine particles (a) and/or the fine particles (b) and the fine particles (c).

## Patentansprüche

1. Bildaufnahmeblatt für den thermischen Übertragungsdruck mit einem Substrat, einer Zwischenschicht und einer Bildaufnahmeschicht, wobei die Zwischenschicht und die Bildaufnahmeschicht in dieser Reihenfolge auf dem Substrat angeordnet sind, dadurch **gekennzeichnet,** daß die Zwischenschicht eine Schicht umfaßt, die
(a) feine Teilchen einer oder mehrerer Arten von wärmehärtenden Harzen und/oder
(b) feine Teilchen einer oder mehrerer Arten von anderen Harzen als den genannten wärmehärtenden Harzen, mit einem Erweichungspunkt von höher als 150°C, und
(c) feine Teilchen eines Polyolefinharzes als Hauptbestandteile
enthält.

2. Bildaufnahmeblatt für den thermischen Übertragungsdruck nach Anspruch 1, dadurch **gekennzeichnet,** daß die Menge der feinen Teilchen (a), die in der Zwischenschicht enthalten sind, im Bereich von 5 bis 90 Gew.-% gegenüber der Gesamtmenge der feinen Teilchen (a) und/oder der feinen Teilchen (b) und der feinen Teilchen (c) liegt.

## Revendications

1. Feuille réceptrice d'images pour l'impression par transfert thermique comprenant un substrat, une couche intermédiaire et une couche réceptrice d'images, cette couche intermédiaire et cette couche réceptrice d'images étant disposées dans cet ordre sur ce substrat, caractérisée en ce que cette couche intermédiaire comprend une couche contenant :
(a) des particules fines d'une ou de plusieurs sortes de résines thermodurcissables et/ou
(b) des particules fines d'une ou de plusieurs sortes d'autres résines que ces résines thermodurcissables, ayant un point de ramollissement supérieur à 150°C et
(c) des particules fines d'une résine polyoléfine, en tant que principaux constituants.

2. Feuille réceptrice d'images pour l'impression par transfert thermique suivant la revendication 1, dans laquelle la quantité de particules fines (a) contenue dans la couche intermédiaire est comprise entre 5 et 90% en poids par rapport à la quantité totale des particules fines (a) et/ou des particules fines (b) et des particules fines (c).
